

## UNITED STATES PATENT OFFICE

JAMES B. RATHER AND LESLIE C. BEARD, JR., OF BROOKLYN, AND ORLAND M. REIFF, OF JACKSON HEIGHTS, NEW YORK, ASSIGNEES TO SOCONY-VACUUM CORPORATION, OF NEW YORK, N. Y., A CORPORATION OF NEW YORK

## DISTILLATE PETROLEUM PRODUCTS AND METHOD OF TREATING SAME

No Drawing. Application filed November 26, 1926, Serial No. 151,005. Renewed December 20, 1930.

This invention relates to distillate petroleum products and to method of treating same to prevent spontaneous discoloration and formation of odor therein.

5 It is well recognized that the distributors and consumers of kerosene and gasoline insist that these products be clear and free from discoloration and odor as an entirely distinct and separate matter from the actual 10 capabilities and usefulness of the products for the ordinary uses for which they are intended. It is also well recognized that kerosene and gasoline spontaneously become unclear, discolored and odorous gradually 15 upon continued exposure to air, thus after a while becoming objectionable to the trade.

The principal object of this invention is to provide a distillate petroleum product, notably kerosene and gasoline, which will 20 remain clear and free from discoloration and odor without impairment or lowering of its effectiveness and capabilities for use; and to provide a simple and inexpensive 25 method of producing distillate petroleum products having the characteristics and qualities referred to.

Other objects of this invention will be in part obvious and in part pointed out hereinafter.

30 In accordance with this invention, the improved product consists of a petroleum distillate, notably kerosene and gasoline, containing a negative oxidation catalyst. The catalyst may be added in the still during 35 distillation, or placed in the condenser in which the distillate is condensed, or the catalyst may be added to the distillate after removal from the condenser, it being advisable, however, to add the catalyst before 40 any appreciable quantity of atmospheric oxygen has been taken up by the distillate, because such oxygen is apt to cause the formation in the distillate of substances which are apt to promote the addition of 45 further oxygen and may tend to offset any advantage to be gained by the subsequent addition of the negative oxidation catalyst.

These objectionable substances, while frequently colorless and odorless, are apt to

undergo change resulting in the development of objectionable color and odor.

The negative oxidation catalyst or catalysts should be of such nature that when added to kerosene or gasoline in sufficient 55 quantities for the purpose they do not effect the color and odor, or materially increase the cost of production, since such effects would raise commercial objections to the product.

60 The following substances and classes of substances constituting negative oxidation catalysts are mentioned as suitable for the treatment above described:

Aromatic amines; for instance, alpha 65 naphthylamine, para phenylenediamine and phenylhydrazine.

Substituted phenols and poly phenols; for instance, cresol and hydroquinone.

Ureas and urea derivatives; for instance, 70 urea and thiourea.

Alkaloids; for instance, brucine and nicotine.

The agents above named which occur in solid form are preferably dissolved in an 75 aliphatic alcohol, for instance, butyl alcohol, or in an aromatic alcohol, for instance, benzyl alcohol, before being applied to the oil. Although all of the above agents and classes of agents can be used in gasoline and 80 kerosene as negative oxidation catalysts, in the practice of this invention we prefer to use a saturated solution of hydroquinone, brucine or nicotine in secondary or tertiary butyl alcohol, the secondary or tertiary 85 butyl alcohol serving to facilitate the solution of the hydroquinone, brucine or nicotine in the oil. The amount of saturated solution of hydroquinone, brucine or nicotine in secondary or tertiary butyl alcohol, properly 90 to be applied to the oil, may vary from 1 part in 5 thousand to 1 part in 50 thousand, depending upon the amount of stabilization desired, the character of the distillate, i.e., its susceptibility to oxidation, and the storage 95 temperature.

We have also produced our invention successfully in a commercial way by dissolving five pounds of hydroquinone in five gallons of isopropyl or secondary butyl alcohol, and 100

adding this solution with appropriate agitation to the petroleum product to be treated, in the proportion of one part of the above solution to from 10,000 to 20,000 parts of the petroleum product, according to the amount of stabilization desired. Oil treated with one part of hydroquinone to 75,000 parts of oil standing for twenty-six weeks at 125° F. has disclosed a discoloration test of 9 points, Saybolt chronometer, as against a deterioration of 24 points of the same oil under exactly the same conditions.

Any of the above mentioned substances are suitable either alone or in combination with others. It is never required to add more than 0.02% to the kerosene or gasoline, and the amount may be as small as 1 part negative catalyst to 500 thousand parts oil. Not over 1 part of brucine or nicotine in 50,000 parts of gasoline or kerosene should be added, as an over-abundance of the agent will tend to cause discoloration of the product.

It will be apparent from the above that this invention is directed primarily to preventing discoloration and formation of odor in the lighter petroleum distillates, notably those of A.P.I. gravity higher than 37 degrees, and particularly kerosene and gasoline. Consumers and distributors of these products require that they be clear and free from discoloration and objectionable odor without considering the question of serviceability for the use intended.

Kerosene and gasoline, however, must be maintained comparatively inexpensive in order to satisfactorily cope with commercial competition, and therefore any treatment must be such that the cost of production is not increased a prohibitive amount. Applicants' method satisfactorily meets this delicate situation since the amounts of negative catalyst the treatment requires are so small that increase in the cost of manufacture and price to the consumer is negligible. At the same time the treated kerosene and gasoline is capable of being stored and handled without danger of its becoming discolored or odorous.

The expression "negative oxidation catalyst" has been used above in its ordinary sense, that is, to mean a substance, usually a compound containing carbon, which retards the attainment of equilibrium in a chemical system in which oxidation is the fundamental reaction.

It is understood that this invention is not intended to be limited to the precise substances mentioned specifically, nor to the exact proportions stated, since applicants have described merely certain possible applications of the invention which are preferred at this time.

Our copending application, Serial No. 315,914, filed October 29, 1928, improve-

ments in distillate petroleum products and method of treating same, includes disclosure of the subject matter of this application and claims certain of the subject matter as to which claims have not been maintained herein.

What we claim is:—

1. The method of preventing discoloration of light colored petroleum distillates in the gasoline-kerosene boiling range which comprises adding thereto a minute amount of an alkaloid. 75

2. The method of treating a light colored petroleum distillate in the gasoline-kerosene boiling range to prevent objectionable discoloration thereof which comprises incorporating into said distillate a minute quantity of an alkaloid of the class described. 80

3. A light colored substantially color stable petroleum distillate in the gasoline-kerosene boiling range having added thereto as a color stabilizer a minute quantity of an alkaloid. 85

4. The method of the character described, which includes adding a minute quantity of a saturated solution of brucine in one of the butyl alcohols to a petroleum distillate to prevent spontaneous discoloration and formation of odor in the distillate. 90

5. A petroleum product consisting of a petroleum distillate containing minute amounts of one of the butyl alcohols and brucine. 95

This specification signed this 23 day of November, 1926.

JAMES B. RATHER.  
LESLIE C. BEARD, JR.  
ORLAND M. REIFF.

100

105

110

115

120

125

130